

Aug. 21, 1928.

1,681,609

J. E. CONZELMAN

PILE AND PROCESS OF MAKING SAME

Filed Jan. 15, 1926

Fig. 1.



Fig. 3.



Fig. 4.



Fig. 6.



Fig. 7.



Fig. 2.



Fig. 5.



INVENTOR:

J. Conzelman,  
by Carl R. Rein  
His ATTORNEYS

Patented Aug. 21, 1928.

1,681,609

# UNITED STATES PATENT OFFICE.

JOHN E. CONZELMAN, OF SOUTH PASADENA, CALIFORNIA.

## PILE AND PROCESS OF MAKING SAME.

Application filed January 15, 1926. Serial No. 81,472.

Reinforced concrete piles have many merits and advantages that are well known; but heretofore their use in sea water has been greatly limited on account of the injurious effect of the sea water thereon. I have observed that such injury is almost wholly limited to the portion of the pile at and adjacent to the water line, where the pile is subject to the conjoint or alternate action of the sea water and the air. The object of the present invention is to minimize the destructive action of the sea water without undue expense, and to provide a pile suitable for use in sea water. The invention consists principally in making a shell suitable for resisting the action of sea water and using said shell as a part of the form in which the pile is cast and as a permanent protector for the water line portion thereof. It also consists in the pile and in the process of making the same hereinafter more fully described and claimed.

In the accompanying drawing which forms part of this specification and wherein like numerals refer to like parts wherever they occur,

Fig. 1 is a longitudinal section of a shell forming part of my invention;

Fig. 2 is a cross-section thereof on the line 2—2 of Fig. 1;

Fig. 3 is a longitudinal sectional view of the shell with a heavy coating or layer of asphaltic or bituminous matter;

Fig. 4 is a longitudinal sectional view of a pile together with the form-work in which it is cast;

Fig. 5 is a cross-section of the finished pile on the line 5—5 of Fig. 6;

Fig. 6 is an elevation of the finished pile;

Fig. 7 is a detail view showing a modified form of joint between the end of the shell and the shoulder of the body of the pile.

In carrying out my invention, a hollow shell of dense concrete suitably reinforced with circumferential reinforcement 2 and longitudinal reinforcement 3 is first made. The longitudinal reinforcement is preferably in the form of bars 3 that project beyond both ends thereof a sufficient distance to be firmly anchored in the concrete of the body portion of the pile, the end portions being preferably hooked to increase the efficiency of such anchorage.

In use it is intended that this shell shall cross the normal range of the water level as such level rises and falls with the waves and

tides; and for this reason it should preferably be made of such length that the portion of the pile above it remains out of the water under normal conditions of waves and tides and the portion of the pile below it remains under the water under normal conditions of waves and tides. One of the functions of the shell is to stiffen the pile by increasing its moment of inertia or resistance; and for this reason the shell should be large enough to permit ordinary handling without breakage. After the pile is set in place, any cracks due to crossbending stresses are most likely to develop below the shell where they are the least destructive.

As this shell is exposed to the full brunt of the action of the sea water, it should be made of dense concrete whether or not it is otherwise especially treated to increase its resistant qualities. After such shell has thoroughly hardened, it is given a thick coat or coats of asphaltic or bituminous matter 4 inside and outside. Preferably, this coating is effected by immersing the shell in asphalt cut or liquefied with gasoline, distillate or the like at atmospheric temperature or in asphalt heated sufficiently to make it quite fluid, whereby the asphalt is enabled to fill the pores of the concrete for an appreciable depth as well as coat the surface thereof. This initial coat is preferably thickened by permitting it to cool and then dipping the shell one or more times in liquid asphalt. The ends of said shell and especially the projecting ends of the reinforced bars are cleaned; and then the shell thus thickly coated with asphalt is placed inside of a suitable form-work or mold 5 in which the main body of the pile is cast.

In the construction illustrated in Fig. 4, the main portion of the mold is preferably of uniform diameter or of uniform taper from the top end to the shoulder near the lower end, and the reinforced concrete shell lies inside of this main mold. The circumferential reinforcement 6 and the longitudinal reinforcement 7 of the body portion of the pile are of any suitable type and are placed in the mold and embedded in the concrete in accordance with suitable practice. In this way, the concrete of the body portion of the pile thoroughly embeds and anchors the portions of the longitudinal bars 3 that project beyond the ends of the shell and causes the shell to contribute greatly to the strength of the pile in resisting cross-bending stress and other stresses due to handling.

In the operation of drying, the concrete of the body portion shrinks slightly longitudinally and thereby exerts considerable compression against the ends of the shell thus closing any circumferential cracks that may have developed in said shell and forming a very tight joint between the ends of the shell and the circumferential shoulders 8 opposite said ends on the body portion of the pile.

10 Preferably the longitudinal reinforcing members of the pile project beyond the top end thereof and are adapted for cooperation with other structural elements.

While I have illustrated the shell of the pile as of the same outside diameter as the outside diameter of the body portion of the pile above and below it, it is obvious that the outside diameter of such shell may be greater than that of the body portion, in which case 20 the inside diameter of the shell may equal the outside diameter of the body portions above and below it.

Obviously my pile has all the advantages of an ordinary pile of reinforced concrete together with special advantages of its own. For instance, the shell of especially dense concrete extends throughout the region that is subject to the destructive action of the salt water and is therefore as efficient in resisting such action as if the entire pile were made of such especially dense concrete. By limiting the effort to resist the action of the water to the region that is exposed to the action of the water, the cost of the pile, which might otherwise be prohibitive, is brought within a practicable limit. Likewise such shell and its reinforcement are located where they greatly increase the strength of the pile; and by limiting the length of the shell, the effect of crossbending stresses is to a large extent confined to the region below the shell where cracks are of relatively slight importance. The making of the resistant portion of the pile in the form of a hollow shell is simple and efficient; and the casting of the body portion of the pile in and around the ends of said shell, after the same is thoroughly coated with asphalt makes it impossible for the water to reach the interior of said shell. By reason of the inside layer of asphalt being so thoroughly protected by the shell, such layer will remain effective even after serious injury to or deterioration of the shell itself.

What I claim is:

1. A reinforced concrete pile wherein the 55 water line part thereof comprises an exterior shell of denser concrete than the body, said shell having longitudinal reinforcement whose ends are embedded in the concrete of the body.

2. A reinforced concrete pile comprising an elongated body portion and a reinforced concrete enclosing shell of denser concrete than said body, said shell terminating short of each end of said body but extending 60 through the region of maximum crossbending 65 stress of the pile considered as a beam and through the normal range of the level of the water surrounding said pile in situ, the outside diameter of said body above and below said shell being greater than the inside diameter of said shell, whereby the shrinking of the subsequently cast body causes it to press against the ends of said shell.

3. A reinforced concrete pile wherein the 75 water line part thereof comprises an exterior shell of denser concrete than the body, said shell constituting a mold for the body and being coated inside and outside with a plastic material that is resistant to the action of salt 80 water.

4. The process of making reinforced concrete piles which consists in first forming and hardening a reinforced hollow shell with reinforcing members extending beyond the ends 85 thereof, coating said shell inside and outside with a thick layer of bituminous matter and then casting the body portion of such pile in a form of which said shell constitutes the portion in which the water-line portion of the 90 pile is cast.

5. A portable reinforced concrete pile wherein the water line part thereof comprises an exterior shell of denser concrete than the body, said shell extending through the region 95 of maximum crossbending stress of the pile considered as a portable beam and through the normal range of the water level when the pile is in situ and terminating short of the ground level, said shell constituting a mold 100 for said body and being reinforced longitudinally throughout its length to resist crossbending stresses.

Signed at Los Angeles, California, this 6th day of January, 1926.

JOHN E. CONZELMAN.